

## 1

3,137,576

## PROCESS OF PRODUCING PHOTOGRAPHIC SILVER HALIDE EMULSIONS UTILIZING SULFONATED POLYPHENYLENE OXIDE

Wolfgang Himmelmann, Cologne-Stammheim, Helmut Mäder, Leverkusen, and Rolf Fred Posse, Cologne-Flittard, Germany, assignors to Agfa Aktiengesellschaft, Leverkusen, Germany, a corporation of Germany

No Drawing. Filed Oct. 16, 1962, Ser. No. 231,004  
Claims priority, application Germany Oct. 25, 1961  
6 Claims. (Cl. 96—94)

The invention relates to a silver halide emulsion and a process for their production.

According to the conventional method, the silver halide is precipitated in gelatine solution and the resulting emulsion thereafter solidified by cooling and the gel is cut into pieces and freed from soluble salts by washing with cold water. On account of the diffusion velocity of the salts, this process necessitates certain rinsing periods. Depending on the nature of the gelatine, the volume of the gel increases to a large or small degree and frequently an undesired lowering of viscosity occurs. This must often be compensated for by adding gelatine during the subsequent melting (ripening or casting). Using this process, it is difficult to vary the ratio between silver halide and gelatine as required.

More modern processes produce emulsions with a high silver content. In such a process, the emulsions are coagulated by adding a precipitant to remove the excess salts, separated from the supernatant aqueous solution containing the salts in dissolved form, washed with water and, after adding more gelatine solution, often also redispersed by adjusting the pH to a predetermined value. It is possible in this way to obviate the rinsing operation which occupies a considerable time. In addition, the emulsion character can be varied greatly and improvements in the photographic properties can be obtained. It is to be remembered that with the conventional method, the gelatine solution must have a minimum concentration of about 2-3% in order to achieve the gelling of the gelatine. The increasing importance of this flocculation process is illustrated by the large selection of variants of the process which have become known in recent times. They differ from one another more especially by the nature of the precipitant.

The oldest method of flocculating gelatino-silver halide emulsions is salt flocculation. An excess of, for example, sodium sulphate is added to the emulsions and the gelatine flocculates out with the silver halide. The disadvantage of this method lies in the great excess of salt which is necessary for a complete flocculation. In addition, such precipitates cannot be washed out with water, since they are easily dissolved again. After the washing process, the emulsions still show a certain conductivity, which is attributed to a high residual content of salts.

Furthermore, organic liquids which are miscible with water and in which the gelatine is insoluble have been proposed for flocculating the emulsions. The disadvantage of this method lies in the fact that there is a high consumption of organic solvents and that various salts which are insoluble in the solvent mixture are also precipitated. It is not possible for the coagulates to be washed out with water, so that it is necessary to use a solvent mixture. Methods which are said to improve the washing-out ability of these methods have also been proposed, but they have the same disadvantages.

Another method of flocculating emulsions consists in chemically converting the gelatine. For example, gelatine can be reacted with phthalic acid anhydride and added to the batch gelatine. The gelatine derivatives

## 2

can be precipitated in aqueous solution at pH 3. However, the production of the gelatine derivatives often leads to difficulties as high pH values (in the region of 10) must be used during the reaction. As a result, some of the gelatine is decomposed. Furthermore, derivatives of this type do not permit the production of highly sensitive emulsions. When using these flocculating agents, the photographic properties of the emulsion are so greatly influenced that these precipitation methods cannot be used on existing and tested emulsion recipes, since they influence the composition of the ripening and inhibiting elements to a large extent. For these reasons, a complete redevelopment of the photographic emulsion concerned is usually necessary. This disadvantage has hitherto prevented the practical use of this process.

There have also been described as flocculating agent, compounds which either form complexes with the gelatine or are even insoluble in water at certain pH values. With the precipitation thereof, the gelatine is also entrained. For example, alkyl-sulphonic acids containing a high number of carbon atoms ( $C_{12}-C_{20}$ ) have been proposed. With the gelatine they form adducts which are insoluble at pH 2-3. A disadvantage in this case is the large amount of the respective sulphonic acids (20-30%) which have to be added, the casting difficulties which are a consequence thereof and the relatively low pH value of the precipitation. It is known from practice in the production of emulsions that the sensitivity of a highly sensitive emulsion decreases as the pH value becomes too acid (<4).

High-molecular acid-insoluble compounds with carboxyl groups have also been proposed as flocculants. In this case, the relatively low flocculation pH value and the modification of the physical properties of the gelatine, for example, the water permeability, the high swelling, the modified adhesion and the impaired redispersability, constitute disadvantages. Benzaldehyde sulphonic acid acetals of polyvinyl alcohol have also been described as flocculants, but these have the disadvantage that the coagulates of the acetalsulphonic acids and gelatine are only formed at pH values below 3. Another process which is known is the precipitation of emulsions of copolymers with vinyl pyridine and unsaturated carboxylic acids, but this process has the disadvantage that relatively large quantities of copolymer are required for precipitating the emulsions, since the pyridine radical becomes ionised in acid solution, whereby the solubility of the coagulate in acid solution increases. Furthermore, the photographic properties of the emulsion are modified in an uncontrollable manner by the pyridine radicals. Finally, it is known to use copolymers of styrene-sulphonic acids for flocculating gelatine, but these have similar disadvantages to those of the aforementioned polymers.

It has now been found that salts of water soluble high molecular weight polyphenylene oxides containing sulphonic acid groups precipitate silver halide emulsion at pH values of 3.5-6. The substances can be used according to the invention for precipitating all types of such emulsions. However, they are especially suitable for emulsions having a low gelatine content and a particularly high silver halide content, such emulsions are characterised by a silver halide gelatine proportion of at least 1 g. silver halide per 1.5 g. of dried gelatine. A precipitation from highly diluted aqueous solution also occurs without it being necessary to add salts or organic liquids. The gelatine is completely precipitated by the substance according to the invention. The photographic properties of the silver halide emulsions or the gelatine compositions are not changed thereby. By means of the process according to the invention, it is possible for any desired silver halide emulsion to be produced substantially more

easily than was possible with the hitherto known processes. The compounds according to the invention are particularly advantageous over prior art because they are capable of almost completely precipitating the gelatine respectively the silver halide. Thus a loss of silver salts is avoided.

Especially suitable for the precipitation of the silver halide emulsions are polyphenylene oxides of the general formula:



in which R<sub>1</sub> to R<sub>6</sub> represent hydrogen atoms or an alkyl radical containing 1 to 3 carbon atoms; A represents a hydrogen atom or a —SO<sub>3</sub>Me-group, but 1 to 3 and preferably 2 neutralised sulphonic acid groups must be present for each formula unit (i.e. for every three phenylene oxide radical); Me represents any desired alkali metal such as sodium or potassium, alkaline earth metal by magnesium or calcium or ammonium cation, for example, ammonium or alkyl ammonium cations and n represents an integer between 3 and 100.

The effect produced by this process was all the more surprising, as salts of polyphenylene oxide sulphonic acids are readily soluble in water and the corresponding sulphonic acids cannot be precipitated by acidification of their solutions or salt solutions. On account of the numerous oxygen bridges, it had to be assumed that large quantities of polyphenylene oxide sulphonic acid are required for precipitating the gelatine. The advantage of this compound is that for completely precipitating gelatine at a pH value of 3.5–6, it is only necessary to use a relatively small quantity, namely 8 to 20% and advantageously 10–12% of the weight of gelatine, so that the flocculate can be washed out extremely satisfactorily and so that the flocculate can be redispersed very quickly and without residue by adjusting the pH value to about 7 and by gently heating the mixture to 35–45° C.

Another discovery which was particularly surprising to the persons skilled in the art was that the compounds according to the invention do not have any deleterious effect on the photographic properties of the silver halide emulsion. This was not to be expected, since, for example, aliphatic polyethylene oxides are known to have strong influence on the sensitivity of photographic emulsions. In the case of the polyphenylene oxides used according to the invention, the sensitivity and the gradation of the emulsion are not changed. The emulsion is only improved by suppressing the fogging, probably due to the possibility of being able to redisperse the coagulate quicker.

The production can be supplied by this method while maintaining the tested emulsion recipes. The procedure adopted is that the silver halide is precipitated in the batch gelatine. 8–20% of a water-soluble salt of polyphenylene oxide sulphonic acid, calculated on the quantity of gelatine used is added to this dispersion. The pH value is then adjusted to between 3.5 and 6. The emulsion coagulates in the form of fine flakes, the size of which can be varied within certain limits by adjusting to a predetermined temperature. Large flakes and coherent coagulates are obtained when working at relatively high temperatures.

After the settlement of the emulsion, the supernatant liquid is removed by decantation and the precipitate is washed several times with cold water. The residue can be redispersed extremely easily and quickly with water at a temperature below 45° C. by adding alkali until a pH value of 7–8 is reached. The required quantity of gelatine is added and the emulsion is ripened. The conventional additives, such as sensitizers, stabilizers and hardeners, can also be added.

According to a modified form of the process, the pH is adjusted to a value of 3.5–4 and the substance is cooled to 1–2° C. above the solidification point of the gelatine. If an aqueous solution of a salt of the polyphenyl sulphonate is added under these conditions, the emulsion precipitates in finely divided form and can be extracted by suction filtering. The redispersion then proceeds even more quickly.

The method referred to can also be used in order to produce new emulsions with extremely high silver halide content.

Furthermore, it is possible to add other layer-forming natural or synthetic polymers after the redispersion. Thus, highly sensitive silver halide layers based on synthetic plastics, for example, polyvinyl alcohol, hydroxyethylcellulose or cellulose esters, can be produced. These were otherwise only obtained with photographically active gelatine.

Larger quantities of polyphenylene oxide sulphonate acids can be added to the emulsions without any photographic defects being caused. In addition, such emulsions have a higher conductivity and do not have such a strong tendency to electrostatic charging. The mechanical strength of the rinsed layers is good.

The sulphonate acids of the polyphenylene oxides have, as yet, not been described in the literature. Polyphenylene oxides are known and they are prepared from the corresponding phenols. Aqueous solutions of p-bromophenols are condensed with sodium hydroxide solution, sodium bromide being split off (JACS 82 (1960), No. 14, page 3632; Journal Polym. Science, vol. XLIX (1961), page 267–275), or the silver salt of the alkylated bromophenol is initially used and thereafter condensed, silver bromide being split off.

According to another method, the corresponding dialkyl phenols are condensed by oxidation, the phenol being dissolved in nitrobenzene and oxygen being introduced in the presence of cuprous salts and pyridine (JACS 81 (1959), page 6335).

The compounds obtained have molecular weights between 1000 and 30,000. The sulphonate acids are preferably obtained by reacting the polyphenylene oxides with the addition compound of sulphur trioxide and 2,2-dichloroethyl ether in dichlorethane. It is, however, also possible to use other sulphonating agents, such as chlorosulphonic acid. The resulting sulphonate acids are very soluble in water.

The following examples are intended to describe the invention, but not to limit it in any way.

#### 50 PRODUCTION OF POLYPHENYLENE OXIDE SULPHONIC ACID

A solution of 65 cc. of ethylene chloride and 13 g. of dichloro-diethyl ether is stirred at –20° C. 2.1 cc. of sulphur trioxide, stabilised with HCl, are added to the mixture. A solution of 5 g. of polyphenylene oxide in 65 cc. of ethylene chloride is slowly added dropwise at –20° C. The mixture is stirred for another 2 hours, it being possible for the temperature to rise to room temperature. The mixture is concentrated to 30 cc. by evaporation and the sulphonate acid is thereafter precipitated with ethylene chloride, suction-filtered and dried (yield: 8 g.). It is thereafter neutralised in a little water with sodium hydroxide solution (SO<sub>3</sub>H group content: 15.7%).

#### 65 SULPHONATION OF THE POLY-2,6-DIMETHYL-1,4-PHENYLENE OXIDE

6.3 cc. of sulphur trioxide stabilised with HCl is introduced dropwise into a mixture of 200 cc. of dichlorethane and 39 g. of 2,2-dichloro-ethyl ether while stirring and at 0° C. The addition compound of sulphur trioxide and 2,2-dichloro-ethyl ether is formed. After cooling the mixture to –20° C., 9 g. of poly-2,6-dimethyl-1,4-phenylene oxide (prepared according to (JACS 81 (1959), No. 23, page 6335)) in 150 ml. of dichlorethane

## 5

are added dropwise while stirring vigorously, the temperature being kept below  $-18^{\circ}\text{C}$ . Stirring is then continued for another 2 hours at  $-20$  to  $-18^{\circ}\text{C}$ . and then the temperature is raised in the course of 2 hours to  $20^{\circ}\text{C}$ . The precipitated sulphonic acid is suction-filtered and washed with dichlorethane and ether. It is then dissolved in water and neutralised with sodium hydroxide solution. Yield of sodium salt: 23 g.,  $\text{SO}_3\text{H}$  group content: 25.3%.

**SULPHONATION OF POLY-2,6-DIETHYL-1,4-PHENYLENE OXIDE**

The sulphonation is effected as above, except that the following quantities are used:

200 ml. dichloroethane  
62 g. of 2,2-dichloro-diethyl ether  
8 ml. of sulphur trioxide  
10 g. of poly-2,6-diethyl-1,4-phenylene oxide in  
100 ml. of dichlorethane

Yield of sodium salt: 15 g.  
 $\text{SO}_3\text{H}$  group content: 21.2%.

*Example 1*

A photographic emulsion is prepared from the following solutions by mixing at  $50^{\circ}\text{C}$ .

**Solution A—**

10 g. of gelatine  
64 g. of potassium bromide  
3.6 g. of potassium iodide  
500 cc. of water

**Solution B—**

80 g. of silver nitrate  
600 cc. of water

4.5 cc. of a 5% aqueous solution of the sodium salt of a poly-2,6-dimethyl-1,4-phenylene oxide sulphonic acid are added to 200 cc. of this emulsion at  $45^{\circ}\text{C}$ . After adjusting the pH value to 3.5-4 with dilute acetic acid or citric acid, a finely flocculated coagulate is formed.

The mixture is cooled to  $20^{\circ}\text{C}$ , the supernatant liquid is poured off and the coagulate is washed with cold water. The coagulate is thereafter redispersed by adding 24 g. of gelatine in 300 cc. of water at  $40$  to  $50^{\circ}\text{C}$ , the pH value being adjusted to 7. The emulsion has the same sensitivity as the emulsion prepared in conventional manner and the gradation has also not changed.

*Example 2*

A photographic emulsion is prepared by mixing the following solutions:

**Solution A—**

1200 ml. of water  
300 g. of silver nitrate  
300 ml. of ammonia solution ( $d=0.91$ )

**Solution B—**

700 ml. of water  
300 g. of potassium bromide  
6 g. of potassium iodide  
70 g. of gelatine

The solution A is added dropwise over a period of 30 minutes at a temperature of  $40$ – $45^{\circ}\text{C}$ . to the solution B while being thoroughly stirred. After cooling to  $30^{\circ}\text{C}$ ., 70 cc. of a 10% aqueous solution of the sodium salt of a poly-2,6-diethyl-phenylene oxide sulphonic acid are slowly added while continuing stirring. The emulsion is approximately neutralised by adding 160 cc. of glacial acetic acid and thereafter flocculated out by further addition of dilute acetic acid until a pH value of 4 is reached. The flocculate is freed from the liquid by decanting and then washed several times in cold water. The pH value is adjusted to 6.6 with dilute sodium hydroxide solution and the flocculate is redispersed by adding 120 g. of gelatine in 1200 cc. of water. The emulsion thus obtained is ripened in the usual manner at  $50^{\circ}\text{C}$ .

## 6

*Example 3*

A photographic emulsion is prepared from the following solutions:

**Solution A—**

100 g. of silver nitrate are dissolved in  
300 cc. of water and  
100 cc. of ammonia solution ( $d=0.91$ ) are added.

**Solution B—**

10 100 g. of gelatine,  
100 g. of potassium bromide and  
10 cc. of 10% potassium iodide solution are dissolved  
in  
600 cc. of water and the mixture is heated to  $40^{\circ}\text{C}$ .

15 The solution A is introduced dropwise over a period of 5 minutes into solution B. After stirring for another 10 minutes, 12 g. of the sodium salt of poly-2,6-diethyl-phenylene oxide sulphonic acid dissolved in 120 cc. of water are added and the mixture is cooled to  $35^{\circ}\text{C}$ .

20 The mixture is approximately neutralised with 95 cc. of 25% sulphuric acid and thereafter the coagulate is obtained by dropwise addition of acetic acid. The most favourable pH range is 3.5–4. The clear solution is decanted off from the flocculate. The flocculate is there-

25 after washed two or three times with cold water. The flakes are redispersed in 500 cc. of water at  $40^{\circ}\text{C}$ . and dilute sodium hydroxide solution is added to adjust the pH value to 7.2. A solution of 200 g. of gelatine in 1.5 litres of water is added and the emulsion is ripened for 30 about 60 minutes at  $50^{\circ}\text{C}$ . By comparison with an emulsion prepared in the usual way, the emulsion hereby obtained does not show any change in its photographic properties.

*Example 4*

35 An emulsion is prepared by mixing the following solutions at  $45^{\circ}\text{C}$ .

**Solution A—**

900 cc. of water  
40 15 g. of gelatine  
100 g. of KBr

**Solution B—**

120 g. of silver nitrate  
1000 cc. of water

45 Solution B is added to solution A and, after cooling the mixture to  $35^{\circ}\text{C}$ ., 15 cc. per 1 litre of emulsion of a 10% solution of the sodium salt of an unsubstituted poly-phenylene oxide sulphonic acid is added. The pH is adjusted to 4.0 to 4.5, and the emulsion flocculates out. It

50 is thereafter decanted and the precipitate is redispersed by adding 35 g. of gelatine in 500 cc. of water after adjusting the pH to 7 and heating to  $40$ – $50^{\circ}\text{C}$ . after the usual ripening, the emulsion obtained does not differ from an emulsion prepared in the conventional way.

55 *Example 5*

A photographic emulsion is prepared from the following solutions:

**Solution A—**

60 100 g. of silver nitrate  
550 ml. of water

**Solution B—**

45 g. of sodium chloride  
65 1200 ml. of water  
12 g. of gelatine

Solution A is introduced dropwise into solution B while stirring vigorously and at a temperature of  $50^{\circ}\text{C}$ . After cooling to  $35^{\circ}\text{C}$ ., 600 ml. of the emulsion thus prepared is adjusted to a pH value of 4.0–4.3 with 3% sulphuric acid. The emulsion is flocculated out and separated by decantation from the supernatant liquid by adding 15 ml. of a 5% aqueous solution of the sodium salt of poly-2,6-diethyl-phenylene oxide sulphonic acid. The soluble salts are removed from the flocculate by repeated-

ly washing with cold water. The flocculate is thereafter redispersed by adding 35 g. of gelatine in 500 ml. of water. This is then heated to 40-50° C. and the pH value adjusted to 7.

*Example 6*

3 samples of a silver halide gelatine emulsion are prepared, using for each sample

280 g. of gelatine  
1200 g. of silver nitrate  
850 g. of potassium bromide  
10 l. of water

The samples are flocculated according to usual methods by the addition of 53 g. of a flocculant in form of a 10% aqueous solution. As flocculants were used for sample A polystyrene sulfonic acid, for sample B benzaldehyde-o-sulfonic acid polyvinyl acetal and for sample C polyphenylene oxide sulfonic acid according to the invention.

After 10 minutes the supernatant liquid is separated by decantation. The content of silver bromide in 1 litre supernatant water is apparent from the following table:

| Sample                     | A    | B   | C    |
|----------------------------|------|-----|------|
| AgBr content..... grams... | 1.01 | 3.3 | 0.21 |

The pH value for the precipitation of 3.5-6 can be adjusted by the addition of mineral acids, such as sulfuric acids or organic acids. Preferred are mono- or polybasic aliphatic acids, such as acetic acid and citric acid.

We claim:

1. A process for the production of photographic silver halide emulsions, which comprises coagulating a silver halide dispersion in an aqueous gelatine solution by adding to said solution at a pH value of about 7 a water soluble salt of a sulfonated polyphenylene oxide, adjusting the pH value to a value of between about 3.5 and 6 by addition of a water soluble acid selected from the class

8  
consisting of mineral acids and organic acids to cause the gelatine to precipitate as a coagulum from the solution, separating the coagulum from the supernatant liquid, washing said coagulum with water and redispersing it at a pH value of at least 7, said sulfonated polyphenylene oxide having the following general formula:



wherein  $\text{R}_1$  to  $\text{R}_6$  represents a member selected from the group consisting of hydrogen and alkyl radicals up to 3 carbon atoms; A represents a member selected from the class consisting of hydrogen and a neutralized sulfonic acid whereby the sulfonic polyphenyl oxide contains 1-3 sulfonic acid groups for each formula unit of three phenylene oxide groupings and  $n$  represents an integer between 3 and 100.

15 2. A process according to claim 1, wherein said sulfonated polyphenylene oxide has a molecular weight between 1000 and 30,000.

3. A process according to claim 1, wherein said sulfonated polyphenylene oxide is added in concentrations of 8-20% based on the dry weight of the gelatine.

25 4. A process according to claim 1, wherein said sulfonated polyphenylene oxide is a sulfonated 2,6-dimethyl polyphenylene oxide.

30 5. A process according to claim 1, wherein said sulfonated polyphenylene oxide is a sulfonated 2,6-diethyl polyphenylene oxide.

6. A process according to claim 1, which comprises coagulating a silver halide dispersion in an aqueous gelatine solution, which contains per 1.5 g. of dispersed gelatine at least 1 g. of silver halide by adding to said solution said sulfonated polyphenylene oxide.

No references cited.